

## UNITED STATES PATENT OFFICE

2,536,685

## SYNTHETIC LUBRICANT

Denham Harman and William E. Vaughan,  
Berkeley, Calif., assignors to Shell Develop-  
ment Company, San Francisco, Calif., a cor-  
poration of Delaware

No Drawing. Application June 2, 1947,  
Serial No. 751,977

8 Claims. (Cl. 252—46.6)

1

This invention relates to novel products and to their preparation and use. More particularly, it pertains to the use of certain sulfur-containing linear polymers especially useful as synthetic lubricants or as lubricant additives.

Mineral oil fractions are suitable for many lubricating purposes, but it is well known that such lubricants possess certain inherent limitations such as tendency to oxidize, thickening at low temperatures and poor inherent lubricating characteristics under conditions of relatively extreme pressure such as in hypoid gear lubrication. A large number of additives have been employed with mineral oils in order to improve these shortcomings with a certain degree of success.

Various synthetic materials have been proposed for use as synthetic lubricants. These include polymers of cracked wax olefins and alkylated aromatics such as alkylated naphthalenes. Some of these are useful for special purposes but, especially if the synthetic lubricants are derived from olefinic sources, they usually possess corrosion and oxidation characteristics limiting their utilization to a substantial degree. Another type of synthetic lubricant which has been investigated is the alkylene oxide polymer type such as polymerized propylene oxide. This latter type of synthetic lubricant is suitable for use only under mild operating conditions. If even moderate extreme pressure conditions are encountered this type of polymeric lubricant fails to function satisfactorily and results in rapid wear of the machinery or engine being lubricated.

It is an object of this invention to provide novel phosphorus containing products. It is another object of this invention to provide a process for the production of such materials. It is a further object of this invention to provide novel synthetic lubricants. A further object of this invention is to provide novel additives for lubricating compositions, said additives providing such compositions with extreme pressure properties. Other objects will become apparent during the following discussion.

Now in accordance with this invention, it has been found that synthetic lubricants having outstanding extreme pressure properties and corrosion characteristics comprise polymers containing units having the general configuration

—(O—R)—

wherein R is an organic radical (especially a hydrocarbon radical) when treated with phosphorus

2

or a phosphorus containing compound. Still in accordance with this invention, it has been found that such polymers add extreme pressure characteristics in an unexpected degree to oxygen-containing oleaginous materials and may be used therewith in substantially any portion. Thus, these phosphorized polymers comprise unusually effective lubricants in themselves or modifiers for oxygen-containing lubricants.

10 Polymers which may be phosphorized for the purpose of the present invention include especially those prepared from alkylene oxides and alkylene glycols.

15 Alkylene oxides, and particularly the alkylene oxides having the oxygen bound to adjacent carbon atoms, form polymers of the above configuration. These monomeric oxides have the general configuration

20



25 wherein the free valences are satisfied with hydrogens or organic radicals.

Alkylene oxides which form such polymers include ethylene oxide, propylene oxide, 1,2-butylen oxide, 2,3-butylen oxide, isobutylene oxide, tetramethylethylene oxide, methylphenylethylene oxide, cyclohexene oxide, methylcyclohexene oxide, 1,2-cetene oxide; and other substances containing the epoxide linkage such as epichlorohydrin, epibromohydrin, and glycidic such as glycidol and 1,2-epoxy-2-butanol, as well as derivatives and polymerizable homologs and analogs of the aforementioned substances.

30 Copolymers of the alkylene oxides useful in compositions of the present invention include for example, the copolymers of ethylene oxide and propylene oxide; and copolymers of ethylene oxide and isobutylene oxide; the copolymers of propylene oxide and epichlorohydrin; the copolymers of propylene oxide and 1,2-butylen oxide; the copolymers of propylene oxide and glycidol; and the copolymers of propylene oxide and iso-  
35 butylene oxide.

40 Polymers similar to those above are formed from the alkylene glycols, including the polymethylene glycols and the ethylene glycols. The monomeric and lower polymeric glycols have the general configuration



50 wherein m and n are integers and the free va-

lences are satisfied with hydrogen atoms or organic radicals. When  $n$  is 1, the general formula is that of an ethylene glycol, wherein the glycolic hydroxyls are on adjacent carbon atoms.

Glycols having three carbon atoms separating the glycolic hydroxyls are derived from 1,3-propanediol (trimethylene glycol) and have the general formula:



wherein  $n$  is an integer and  $\text{R}_1$  and  $\text{R}_2$  are hydrogens or organic radicals.

If  $\text{R}_1$  and/or  $\text{R}_2$  are not hydrogen atoms, they may be organic radicals such as alkyl, aralkyl, aryl, etc. Preferably, if they are not hydrogens, they are aliphatic radicals, especially saturated lower aliphatic radicals, but may also be groups which contain olefinic or acetylenic links. Typical of the trimethylene alkyl substituted glycols are the methylated trimethylene glycols, including 1-methyl-1,3-propanediol; 2-methyl-1,3-propanediol; 1,1-dimethyl-1,3-propanediol; 1,2-dimethyl-1,3-propanediol; 1,3-dimethyl-1,3-propanediol; 2,2-dimethyl-1,3-propanediol; 1,1,2-trimethyl-1,3-propanediol; 1,1,3-trimethyl-1,3-propanediol; 1,2,2-trimethyl-1,3-propanediol; 1,2,3-trimethyl-1,3-propanediol; 1,1,2,2-tetramethyl-1,3-propanediol; 1,1,3,3-tetramethyl-1,3-propanediol; 1,2,3,3-tetramethyl-1,3-propanediol; 1,1,2,2,3-pentamethyl-1,3-propanediol; 1,1,2,3,3-pentamethyl-1,3-propanediol; and hexamethyl-1,3-propanediol.

In place of the methyl groups other alkyl groups may be utilized such as ethyl, propyl, butyl, amyl, hexyl, heptyl, octyl, nonyl, decyl, etc., as well as their isomers. Preferably, when alkyl groups are the substituents  $\text{R}_1$  and  $\text{R}_2$ , they have from 1 to 10 carbon atoms, and still more preferably from 1 to 5.

It will be understood that  $\text{R}_1$  and  $\text{R}_2$  may be similar or dissimilar groups. Thus, when expanding the general formula given hereinbefore to its indicated number of carbon atoms, it then becomes



wherein  $\text{R}_3$  through  $\text{R}_8$  are either hydrogen atoms or similar or dissimilar organic radicals. Those derivatives of trimethylene glycol, other than trimethylene glycol itself, which gives the most satisfactory polymers for general use have either one or two of the  $\text{R}'s$  as lower alkyl groups. Thus, 2-methyl-1,3-propanediol and 2,2-dimethyl-1,3-propanediol form excellent polymers when treated according to the method of the present invention.

Other lower alkyl substituted trimethylene glycols which polymerize readily are 1-methyl-2-ethyl-1,3-propanediol; 2-methyl-2-ethyl-1,3-propanediol; 1-methyl-3-ethyl-1,3-propanediol; 2-methyl-2-propyl-1,3-propanediol; 1-methyl-2-isopropyl-1,3-propanediol; 2-methyl-2-butyl-1,3-propanediol; 2-methyl-3-butyl-1,3-propanediol; and the homologs, analogs and derivatives of the same.

Cycloaliphatic radicals may be one or more of the substituents represented by  $\text{R}_3$  to  $\text{R}_8$  in the above general formula. Thus  $\text{R}_3$  through  $\text{R}_8$  may be such radicals as cyclohexyl, methylcyclohexyl, dimethylcyclohexyl, ethylcyclohexyl, etc. How-

ever, open chain alkyl substituents form polymers having preferred properties.

The polymers have modified properties if the trimethylene glycol derivative contains other active groups, such as additional hydroxyls, carboxyls, carbonyls, halogens, sulfur, phosphorus, nitrogen, etc.

Polymethylene glycols having 6 or more carbon atoms separating the glycolic hydroxyls also form polymers and copolymers which are readily treated as described herein.

The polymethylene glycols from which such polymers are prepared have the general formula



wherein  $Z$  is an integer,  $y$  is an integer greater than 5 and the  $\text{R}'s$  are substituents attached to each carbon atom, such as hydrogen atoms or organic radicals, especially hydrocarbon radicals. Preferably  $Z$  is an integer less than 10, and more preferably is an integer between 1 to 4. Actually, when  $Z$  is more than 1, the glycol is a dimer, trimer, etc., of the corresponding monomeric glycol. The polymethylene glycols polymerizing most readily are those in which  $y$  is an integer from 6 to 20.

Monomeric, unsubstituted polymethylene glycols falling within the above formula include 1,6-hexanediol; 1,7-heptanediol; 1,8-octanediol; 1,9-nonanediol; 1,10-decanediol; 1,12-dodecanediol; and polymerizable homologs, analogs and derivatives of the same.

The above glycols are those in which all of the  $\text{R}$  substituents attached to the carbon atoms are hydrogen atoms. When one or more of the  $\text{R}'s$  are substituents other than hydrogen atoms they may be hydrocarbon radicals, such as aliphatic, aromatic, or alicyclic hydrocarbon radicals, or radicals containing non-hydrocarbon members, such as hydroxyl, carboxyl, or carbonyl groups, or sulfur, selenium, tellurium, phosphorus or nitrogen atoms. Preferably, however, any organic radicals attached to the polymethylene glycol are hydrocarbon radicals. Of these, the aliphatic hydrocarbons are preferred, and the saturated lower aliphatic radicals give the most stable polymers and have the widest utility. Hence, the preferred  $\text{R}'s$ , other than hydrogen, are the lower alkyls, such as methyl, ethyl, propyl, isopropyl, butyl, secbutyl, tertbutyl, amyl, isoamyl, hexyl, etc. groups. Again even when  $\text{R}'s$  other than hydrogen are present, it is preferred that the monomeric glycol contain a preponderance of hydrogen substituent  $\text{R}'s$ . The most reactive glycols are those in which less than 4  $\text{R}'s$  are other than hydrogen, and the greatest reactivity is possessed by those having 2 or less  $\text{R}'s$  which are organic radicals.

Glycols which fall within the above classification include 1,6-heptanediol; 1,6-octanediol; 1,6-nonanediol; 1,6-dodecanediol; 1,6-decanediol; 1,7-octanediol; 1,7-nonanediol; 1,7-decanediol; 1,7-dodecanediol; 1,8-nonanediol; 1,8-decanediol; 1,9-decanediol; 1,9-dodecanediol; 1,10-dodecanediol; 2,7-octanediol; 2,7-nonanediol; 2,7-decanediol; 2,7-dodecanediol; 2,8-nonanediol; 2,8-decanediol; 2,8-dodecanediol; 2,9-decanediol; 2,9-dodecanediol; 2,3-dimethyl-1,6-hexanediol; 2,4-dimethyl-1,6-hexanediol; 2,5-dimethyl-1,6-hexanediol; 4,4-dimethyl-1,6-hexanediol; 5,5-dimethyl-1,6-hexanediol; 2-methyl-3-ethyl-1,7-heptanediol; 2-ethyl-3-

methyl - 1,7 - heptanediol; 3,3-diethyl-1,7-heptanediol; 3,4 - diisopropyl-1,8-octanediol; etc., and their polymerizable homologs, analogs and derivatives.

The polymers described hereinbefore may be homopolymers or may be copolymers. For example, an ethylene glycol may be copolymerized with a trimethylene glycol to give copolymers having units of the general configuration:



wherein  $m$  and  $n$  are integers and the free valences within the brackets are satisfied with hydrogen atoms or organic radicals. These include copolymers of ethylene glycol and trimethylene glycol; ethylene glycol and 1-methyl-1,3-propanediol; ethylene glycol and 2-methyl-1,3-propanediol; ethylene glycol and 2,2-dimethyl-1,3-propanediol; ethylene glycol and 1,3-diethyl-1,3-propanediol; 1,2-dimethylethylene glycol and trimethylene glycol; 1,2-dimethyl-ethylene glycol and 1,3-dibutyl-1,3-propanediol, etc.

Other copolymers falling within the general formula of substances stabilized according to the present invention include the copolymers of an ethylene glycol or a trimethylene glycol with a polymethylene glycol having more than 5 carbon atoms separating the glycolic hydroxyls. These copolymers have units of the general configuration:



wherein  $m$ ,  $n$ ,  $p$  and  $y$  are integers, and the free valences are satisfied with hydrogen atoms or organic radicals. These include for example, copolymers of ethylene glycol and hexamethylene glycol, trimethylene glycol and hexamethylene glycol, etc.

The alkylene oxides usually are polymerized at temperatures from about -60° C. to about 100° C. in the presence of alkalies, acids, amines, or salts. The glycols are polymerized at higher temperatures (100-300° C.) in the presence of dehydration catalysts, such as iodine, mineral acids, such as nitric acid or sulfuric acid, hydrogen halides such as hydrogen iodide or hydrogen chloride; or organic sulfonic acids such as para-toluene sulfonic acid.

In producing the phosphorized polymers for use as lubricants or as modifiers for oxygen-containing lubricants it is preferred practice to heat one or more of the polymers at a temperature from about 50° C. to about 200° C. for a period of about 3 hours with an agent selected from the group consisting of phosphorus, phosphorus halides and phosphorus oxyhalides. Suitable halides include especially phosphorus trichloride, while the most effective oxyhalide is phosphorus oxychloride. However, the iodides, bromides and fluorides as well as the corresponding oxyhalides may be used for the present purpose. The reaction mixture may be heated in the absence of other materials or in the presence of solvents for one or more of the ingredients or products.

An especially suitable means of preparing the subject lubricants comprises heating a large excess of the polymer with phosphorus or a phosphorus compound in such a manner that only a minor amount of the product obtained has been phosphorized while the remainder is in an unmodified condition. Thus lubricants having

any predetermined degree of extreme pressure characteristics may be prepared.

In carrying out the preparation of these phosphorized lubricants therefore, any desired degree of phosphorization may be effected by controlling the ratio of phosphorus or phosphorus compound to the polymer. Preferably the amount of phosphorus in the product will vary from about 1% to about 20% by weight of the polymer. However, higher or lower percentages may be employed. In order to obtain a synthetic lubricating material having satisfactory extreme pressure properties at high loads it is usually preferred that the percentage of phosphorus be from about 3% to about 10%, based on the weight of the polymer.

Under normal operating conditions it is advisable to employ an amount of phosphorus in excess of that amount with which it is desired to modify the polymer. By the use of such an excess the rate of reaction is increased to a satisfactory degree. If an excess is used it becomes necessary at the end of the heating period to separate the unreacted phosphorus or phosphorus compound from the modifier polymeric material. Ordinarily the excess agent will remain in suspension and may be separated by a filtration or centrifuging operation. Under some conditions, however, the excess agent dissolves in the polymer and, if it is necessary to separate therefrom, it must be removed by such means as solvent extraction. For many lubricating purposes an excess of phosphorus is not objectionable if it is dissolved in the body of the lubricant.

The phosphorizing operation normally may be effected without undue discolorization or other adverse effects on the subject polymers. However, it may be desirable to colorize or decolorize the product by subjecting it to an operation such as filtration through activated carbon, treatment with an absorbent clay or by chemical means of decolorization.

The products obtained by the phosphorization of polymers, such as those described above, are solids or liquids useful for a number of purposes. The solids are particularly effective as extreme pressure additives in oxygen-containing lubricants, while the liquid members of the phosphorized series are effective not only as extreme pressure additives but as lubricants themselves. The oily products have satisfactory lubricating characteristics, having high viscosity indices and low pour points.

Lubricants which  $n$  or  $y$  be modified by the addition of a solid or liquid phosphorized polymer as described hereinbefore include oxygen-containing oleaginous materials such as fatty oils; vegetable oils such as corn oil, cottonseed oil and castor oil; animal oil such as neat's-foot oil; and fish oils such as sperm oil. Oleaginous materials when modified by such means as halogenation, hydrogenation, alkylation and other means may be modified by the phosphorized polymers of the present invention. Depending upon the application intended, oleaginous materials of extreme low or extreme high viscosities may be used successfully. Lubricating oils having a viscosity from about 30 seconds at 100° F. to about 250 seconds at 210° F. and higher may be used if desired.

A special type of lubricant which is particularly suited to modification with the subject phosphorized polymers includes lubricants comprising or derived from the alkylene oxide or alkylene glycol polymers listed above. These polymers

7  
may be the same the polymers from which the phosphorized materials are derived or they may be different members of the same class.

The lubricating compositions of this invention may contain other modifying ingredients such as gelling agents, stabilizers, anti-corrosion agents, viscosity index improvers, thickener, and the like. Particularly suitable gelling agents for polymeric alkylene oxides or glycols which contain or comprise sulfurized polymers are lithium soaps of the higher fatty acids such as lithium stearate.

The use of these phosphorized polymers either in or as lubricants is particularly suitable where extreme pressure or heavy duty conditions prevail. It has been discovered that by the phosphorization as described hereinabove pressure characteristics are imparted to the alkylene oxide and glycol polymers. The examples which follow describe the preparation and use of this invention. It is not intended that the invention be limited specifically to these examples but that they be treated as specific illustrations thereof.

*Example I*

100 parts of a polymerized propylene oxide were heated with 5 parts by weight of phosphorus trichloride at a temperature of 170° for 3 hours. The product was filtered and was found to have the following characteristics:

|                               |      |
|-------------------------------|------|
| Phosphorus, percent by weight | 1.42 |
| Chlorine, percent by weight   | 1.16 |
| Viscosity index               | 149  |
| Pour point, °F.               | -30  |

*Example II*

100 parts of a polymerized propylene oxide were heated with 5 parts by weight of phosphorus oxychloride at a temperature of 190° for 3 hours. The product was filtered and was found to have the following characteristics:

|                               |      |
|-------------------------------|------|
| Phosphorus, percent by weight | 1.26 |
| Chlorine, percent by weight   | 1.66 |
| Viscosity index               | 140  |
| Pour point, °F.               | -25  |

*Example III*

The propylene oxide polymer and the phosphorized product thereof formed as described in Examples I and II were tested for extreme pressure properties, using the 4-ball machine described by Boelage in "Engineering" (July 14, 1933). The following data were obtained.

| Lubricant                              | Wear in mm. at Various Loads (kgs.) |      |      |      |      |      |     |     |     |     |
|----------------------------------------|-------------------------------------|------|------|------|------|------|-----|-----|-----|-----|
|                                        | 60                                  | 80   | 100  | 140  | 200  | 300  | 400 | 500 | 600 | 700 |
| Polymerized:                           |                                     |      |      |      |      |      |     |     |     |     |
| propylene oxide                        | 0.57                                | 1.63 | 2.50 | W    |      |      |     |     |     |     |
| propylene oxide +<br>PCl <sub>3</sub>  |                                     | 0.48 | 0.58 | 0.65 | 1.79 | W    |     |     |     |     |
| propylene oxide +<br>POCl <sub>3</sub> |                                     |      | 0.60 | 0.73 | 0.93 | 1.15 | W   |     |     |     |

W indicates welding.

We claim as our invention:

1. As an extreme pressure agent suitable for

imparting extreme pressure properties to oxygen-containing lubricating oils, the reaction product of a propylene oxide polymer with a phosphorus halide, said product having both phosphorus and halogen substituents, the composition having a phosphorus content of 1-20% and a chlorine content of at least 1%, said reaction product being obtained by heating a propylene oxide polymer and a phosphorus halide at a temperature between 50 and 200° C.

2. The process for the preparation of an extreme pressure lubricant which consists essentially of heating 100 parts by weight of propylene oxide polymers with 5 parts by weight of phosphorus trichloride for 3 hours at a temperature of 170° C.

3. The process for the preparation of an extreme pressure lubricant which consists essentially of heating 100 parts by weight of propylene oxide polymers with 5 parts by weight of phosphorus oxychloride for 3 hours at a temperature of 190° C.

4. As an extreme pressure agent suitable for imparting extreme pressure properties to oxygen-containing lubricating oils, the reaction product prepared according to the process of claim 2.

5. As an extreme pressure agent suitable for imparting extreme pressure properties to oxygen-containing lubricating oils, the reaction product prepared according to the process of claim 3.

6. The process for the preparation of an extreme pressure lubricant which consists essentially of heating polyoxyalkylene fluids at a temperature between 50° C. and 200° C. with a phosphorus halide, the proportion of said phosphorus halide being sufficient to impart a phosphorus content to the reaction product of the agent and fluid of between 1% and 20% by weight of the fluid.

7. As an extreme pressure agent suitable for imparting extreme pressure properties to oxygen-containing lubricating oils, the reaction product prepared according to the process of claim 6.

8. An extreme pressure lubricating composition consisting essentially of an oxygen-containing lubricating oil and a reaction product prepared according to the process of claim 6, the proportion of said reaction product being sufficient to impart extreme pressure properties to said composition.

DENHAM HARMAN.  
WILLIAM E. VAUGHAN.

REFERENCES CITED

The following references are of record in the file of this patent:

| UNITED STATES PATENTS |               |               |
|-----------------------|---------------|---------------|
| Number                | Name          | Date          |
| 2,241,243             | Conary et al. | May 6, 1941   |
| 2,241,244             | Conary et al. | May 6, 1941   |
| 2,372,244             | Adams et al.  | Mar. 27, 1945 |
| 2,423,844             | Morgan et al. | July 15, 1947 |